

DANIEL F. FERNEY, OF GRAND RAPIDS, MICHIGAN

## GLUE OR ADHESIVE.

1,235,784.

Specification of Letters Patent.

Patented Aug. 7, 1917.

No Drawing.

Application filed June 8, 1916. Serial No. 102,537.

106-79

*To all whom it may concern:*

Be it known that I, DANIEL F. FERNEY, a citizen of the United States, residing at 840 Butterworth street, Grand Rapids, 5 county of Kent, State of Michigan, have invented certain new and useful Improvements in Glue or Adhesive, of which the following is a specification.

This invention relates to improvements in 10 glue or adhesive.

My improved glue is especially desirable and primarily intended by me for use in the securing of fabrics, leather and the like to metal, such for example as the felt cushion facings to sanding drums or fabric or leather to pulleys or to glass or wood and various other articles. My improved glue is also adapted and suitable for various other uses where ordinary glue is employed.

20 The main objects of my invention are:

First, to provide an improved glue or adhesive which will effectually adhere to metal, glass and like surfaces, so that fabric, leather, rubber and the like may be secured to and effectively retained thereon.

Second, to provide an improved glue or adhesive which has great strength.

Further objects will definitely appear from the detailed description to follow.

30 The invention is clearly defined and pointed out in the claims.

In the preparation of my improved glue I use the following ingredients preferably in about the proportions stated: liquid glass 35 75 parts, gum arabic 2 parts, lye extracted from hard wood ashes 3 parts, milk skinned or milk with the fat removed 10 parts, vinegar, preferably cider vinegar 10 parts. Coloring matter is preferably added but this is 40 optional.

These ingredients are preferably combined by mixing the vinegar, and lye and the gum arabic and then adding the liquid glass and skinned milk thereto. If desired 45 casein and water may be added in lieu of the skinned milk.

If the glue is too thick for easy application it can be thinned to proper consistency by the addition of water without detriment 50 thereto, in fact I prefer to use it quite thin. Further should it become thick by evaporation it may be thinned to proper consistency by the addition of water.

The ingredients should be thoroughly 55 mixed and should be remixed if allowed to

stand for a considerable period before application.

My improved glue or adhesive is particularly desirable and is primarily designed by me for use in securing fabric, leather, 60 rubber or the like to metal, glass or wood, and it is particularly advantageous in the securing of felt covering to sanding drums and the like as the felt is so secured that it cannot loosen or wrinkle in use as is likely 65 to result with the ordinary means in securing such felts.

My improved adhesive is also well adapted for the securing of fabric, rubber, leather and the like to pulleys. The addition of 70 hard wood ashes to the glue makes a very effective cement for use in building up crowns on pulleys and the like, a fabric such as cheesecloth being used in connection therewith and wrapped around and around the 75 pulley with the repeated applications of the glue or cement. By this means, the desired crown can be built up on the pulley and a very superior anti-slip surface provided therefor.

80 A further advantage of my improved glue is that while it is very efficient in the securing of fabrics to iron, glass or wood, when it is desired to remove the same, water is applied, preferably hot water, leaving the 85 article practically clean for the re-application of a new facing.

My improved adhesive is not only very desirable for the securing of fabrics or the like to iron, glass and the like but is desirable for and very superior for use where glue is employed. The same is not, however, designed or intended for use where subjected to the action of water as it is not 90 waterproof and softens or dissolves under 95 the action of water.

A satisfactory way of using, for example, in securing fabric to metal is to apply the glue to the metal and allow it to become somewhat tacky before applying the fabric. 100 Time should be given to permit the glue to fully set before using the article.

While I preferably combine the ingredients in the proportions indicated they may be quite considerably varied and quite desirable results still be secured. I preferably use cider vinegar as acid vinegar does not secure so satisfactory a product. While I 105 preferably combine the ingredients in approximately the proportions specified the 110

proportion may be varied and a desirable product still be secured although the character of the product is more or less affected by such variations.

5 Having thus described my invention, what I claim as new and desire to secure by Letters Patent is:—

1. A glue or adhesive the constituent ingredients of which are liquid glass, 75 parts, vinegar 10 parts, skim milk 10 parts, gum arabic 2 parts, and lye extracted from hard wood ashes 3 parts combined into a mixture.

2. A glue or adhesive the constituent ingredients of which are liquid glass, gum 15 arabic, vinegar, lye, and casein combined in proportions substantially as specified, the said glue, when set, being soluble in water.

In witness whereof, I have hereunto set my hand and seal in the presence of two 29 witnesses.

DANIEL F. FERNEY. [L.S.]

Witnesses:

MARY A. FERNEY,  
JOSEPH RENIHAN.